

# UNITED STATES PATENT OFFICE.

ROBERT IRVINE, OF ROYSTON GRANTON, COUNTY OF MID-LOTHIAN, NORTH BRITAIN.

## LUBRICATING COMPOUND.

SPECIFICATION forming part of Letters Patent No. 242,828, dated June 14, 1881.

Application filed December 6, 1880. (No specimens.) Patented in Great Britain July 29, 1880.

*To all whom it may concern:*

Be it known that I, ROBERT IRVINE, a subject of the Queen of Great Britain and Ireland, and residing at Royston Granton, county of 5 Mid-Lothian, North Britain, chemical manufacturer, have invented certain Improvements in the Manufacture or Production of Lubricating Compounds, (for which I have obtained a patent in Great Britain, No. 3,116, dated July 29, 10 1880,) of which the following is a specification.

This invention relates to the combination of certain oils with the ingredients hereinafter mentioned so as to produce a mixture or compound which possesses improved lubricating 15 properties.

In carrying out my invention I take such oils as are derived by distillation from coal, shale, or other bituminous minerals, or from earth or rock oils, known as "petroleum," or otherwise, 20 or from earth wax or waxes, known as "ozocerite," "bitumen," "asphaltum," or such portions of these oils as are suitable for lubricants, or I employ earth or rock oils which are used in their natural state as lubricants, or mixtures 25 of these several oils, as also residuum from oils known as "oil-residuums" or "still-bottoms," and dissolve in or combine with any one or any mixture of these oils compounds consisting of a fatty acid or fatty acids with an alkali, 30 alkalies, salts having alkaline reactions, and in some cases alkaline earths. This combination or compound, when combined or mixed with water, is commonly known as a "soap" or "soaps." I employ such after the water 35 usually present has been driven off by heat, or after the compound has been otherwise dehydrated, or I employ combinations of fatty acid or acids with alkali, alkalies, salts having alkaline reaction, or alkaline earths heated together in a dry state until combination is effected, or I employ substances containing fatty acids, in combination with glycerine, such as 40 tallow and other animal fats and waxes, vegetable fats or waxes, the same, when decomposed by an alkali, alkalies, salts having an 45 alkaline reaction, or alkaline earths, yielding a soap or saponaceous compound, or these may be heated together with the oils hereinbefore mentioned, so that their combination may be 50 thus effected.

In order to effect the solution of the soap, soaps, or saponaceous matters in the oil, heat is employed, applied at temperatures varying according to the proportions of saponaceous matter added, and ranging up to the boiling-point of the oil or oils heated. 55

When the ingredients of the soap, soaps, or saponaceous matter are in their proper proportions—that is to say, in their chemical equivalents or combining proportions—complete solution or mixture or combination takes place in the oil or oils employed, and hereinbefore described, and the mixture or compound assumes a plastic or greasy structure or consistency at temperatures ranging from 100° 60 Fahrenheit to 260° Fahrenheit and higher, according to the proportion of soap or soaps or saponaceous matter used. 65

By this invention I obtain a plastic or greasy mixture or compound in a solidified form free 70 from water, which is eminently well adapted for preventing friction of rubbing-surfaces, and by minimizing the quantity of soap used I obtain in lieu of a solid product an oil of a greatly increased body which is available for like purposes. 75

The following examples are given as types of the lubricating compounds which may be produced according to my invention. In the practical manufacture of these lubricating compounds 80 I employ varying proportions of saponaceous matters. For example, in order to produce the lubricant having a very high melting-point, I prefer to use a potash soap which has been previously (or is in the process of manufacture) deprived of all water in the proportion of from ten to twenty per cent. This proportion dissolves in or is absorbed by the oil at a temperature of, say, from 300° to 400° Fahrenheit, and produces the lubricant which remains solid at temperatures over 300° Fahrenheit. When not wanted with so high a melting-point I use a less proportion, varying from, say, three to ten per cent., which gives the material with a lower or higher melting-point at 85 will. When it is desired simply to increase the body of a mineral oil I use a minimum quantity of saponaceous matter, varying from, say, one-half to two and one-half per cent. In this case the oil does not become a solid mass, 90 95 100

but retains its liquidity, although the body or viscosity becomes much greater.

It is obvious that in all cases it is necessary to employ a higher temperature in the solution 5 of the saponaceous matters than is required as the melting-point of the resulting product.

I claim as my invention—

The method of making lubricating compounds by dissolving and uniting under the 10 action of heat saponaceous matter and mineral oil, said saponaceous matter comprising a fatty acid and an alkali and being free from water

when added to the mineral oil, substantially as described.

In testimony whereof I have signed my name 15 to this specification in the presence of two subscribing witnesses.

ROBERT IRVINE.

Witnesses:

GEO. HUTTON,  
*Consular Clerk, Leith.*

D. BALFOUR,  
*8 York Buildings, Edinburgh, Law Clerk.*